

Dec. 21, 1965

J. W. SMITH

3,224,897

METHOD AND APPARATUS FOR PRODUCING CAST COATED PAPER

Filed Aug. 19, 1960



FIG. 1



FIG. 2

INVENTOR.

JOHN W. SMITH

BY

ATTORNEY

1

3,224,897

**METHOD AND APPARATUS FOR PRODUCING  
CAST COATED PAPER**

John W. Smith, Chillicothe, Ohio, assignor to The Mead Corporation, Dayton, Ohio, a corporation of Ohio  
Filed Aug. 19, 1960, Ser. No. 50,635  
7 Claims. (Cl. 117—64)

This application is a continuation-in-part of application Serial No. 648,227, filed March 25, 1957, now U.S. Patent No. 2,950,214, dated August 23, 1960.

This invention relates to a process for producing high gloss cast surfaced mineral coated papers, and more particularly to apparatus which provides coat weight control, coat weight level as well as outstanding smoothness of the coated surface and coverage of the rawstock for practicing the process.

In general, cast-surfaced coated papers are coated with pigment coatings in aqueous dispersion. And known commercial apparatus used in processes for applying these coatings includes a plurality of rolls arranged in various configurations. However, such roll coating apparatus has a commonly recognized deficiency in the fact that the fluid coating is split in the application nip where the paper is separated from the roll after coating, and this splitting of the coating produces a rough, piled surface which, even after a casting operation, exhibits objectionable surface defects.

Numerous unsuccessful attempts have been made to correct this deficiency by adopting so-called standard reverse roll processes used for applying pigmented printing coatings to paper on large scale machine operations. But the inability to meter the thin films required to produce the desired weights of pigmented coatings appears to be the crux of the problem. When using water system as in cast coating operations, where surface tension forces are higher than in organic solutions, and when the film thickness on the casting roll becomes too thin, or when the casting roll is run too slowly with respect to the paper backing roll, and when the coating color viscosity is low at the same time, or is too low per se, the film on the surface of the casting roll tends to become unstable. Surface tension forces cause the film to buckle or draw into droplets, and the coating applied to the web is non-uniform in thickness or is actually discontinuous.

Further limitations of conventional reverse roll coaters used in processes of making mineral coated paper involve difficulties in fabricating metal roll surfaces, and in providing supports for the rolls with sufficient precision to meter the necessary thin films for cast coating. For example, in metering a film 0.010 inch thick, which is the proper range for functional coating, a variation of 0.001 inch represents only 10 percent. The same variation would be 100 percent of a film only 0.001 inch thick, which is the range used for pigmented coating. So thin are the films of normal pigmented coatings, that even localized variations in the temperature of the faces of two metal metering rolls produce significant changes in the meter film thickness. Moreover, known present forms of reverse roll coaters are only adapted to narrow deckles because of film thickness difference caused by sagging of the rolls between supports when the supports are very far apart. A further limitation of standard reverse roll coaters is that grit is able to lodge in the metering nip and cause scratches in the coating applied to paper. And since limitations are always present when applying desired low coat weights needed for acceptable printing coatings, reverse roll metering systems have not heretofore been considered acceptable for producing high gloss cast surfaced mineral coated paper.

In accordance with the present invention, a reverse roll

2

coating apparatus is provided for the process of making cast surface mineral coated paper, which apparatus provides an adequate and unexpected metering system. Moreover, it has been found that such a system is capable

5 of producing on the casting roll stable, thin films from high solids, viscous mineral coating compositions, over a wide range of coat weights, without restricted deckle, and with freedom from grit defects. In the practice of this invention, the highly viscous, high solids coating compositions have the effect of stabilizing thin films so that surface tension cannot produce irregularities in thickness of the film on the casting or applicator roll. Moreover, film stability on the applicator roll is required and obtained by this invention whereby a smooth coating is applied to the paper.

10 While conventional reverse roll metering systems cannot use high solids viscous colors because of the excessively high coat weights which would result, the metering system of this invention is adapted to such colors. And 15 the metering system of this invention when combined with a reverse turning applicator roll to continuously apply the coating composition to a paper web without splitting the film is believed to represent a paramount advance in the art.

20 Accordingly, it is an object of the present invention to utilize a reverse roll coater system in the production of high gloss cast-surfaced mineral coated paper.

25 It is a further object to provide such a reverse roll system which insures precise coat weight control, unrestricted 30 coat weight level and excellent smoothness of the coated surface and coverage of the rawstock.

35 Another object is to provide a metering system which is adapted for metering high solids viscous material coating compositions and can be used with a reverse turning applicator roll to apply the coating to paper without splitting the coating film.

40 It is a further object to provide a metering system for the production of high gloss cast-surfaced mineral coated paper, which system is capable of producing on the casting roll stable, thin films of high solids, viscous coating colors, over a wide range of coat weights, without undue sensitivity to changes in the position of the rolls, with unrestricted deckle, and with freedom from grit defects.

45 Numerous other objects of this invention will more fully hereinafter appear.

In the drawings, which illustrate apparatus embodying, and found satisfactory for practicing and effectuating the inventions hereof—

50 FIGURE 1 is a diagrammatic view in side elevation showing apparatus constructed in accordance with and for carrying out the practicing of the present invention; and

55 FIGURE 2 is a modification of the coating apparatus used for carrying out the practicing of the present invention.

60 As shown in FIGURE 1, the paper web to be coated is drawn from roll 10 of suitable paper base stock, and the web 11, is led over guide rolls 12 and 13 to pass through the apparatus in the coating color applying zone.

65 In the modification of FIGURE 1, the web passes through the nip of the coating application rolls 14, 15 where a predetermined amount of coating suspension is applied thereto and distributed with sufficient uniformity over the web surface to give the desired weight of coating material per unit area on the web.

70 The coating color is fed through a suitable supply line and by suitable means to one or more discharge pipes or nozzles 23 and into the nip between roll 15 and metering roll 24 which have the direction of rotation as indicated, the color forming a pool 25. Doctor 26, as shown, functions to maintain the pool in the nip between

rolls 15 and 24 and any well known doctoring means may be employed.

The coated web is then brought with the coated side out tightly around roll 16 which dips into a coagulant and release agent both contained in a tub 17 as described in co-pending Smith application, Serial No. 648,227 filed March 25, 1957, now U.S. Patent No. 2,950,214. The coated paper 11 is then transferred by press roll 18, after the coating has been formed into a non-tacky tough deformable gel, into nip 19, and thereafter into contact with a heated finishing roll 20 having a smooth casting surface. The coating on web 11 remains in contact with casting roll 20 until the coating spontaneously releases therefrom after it has substantially dried and is removed by tension roll 21 to winder roll 22.

In order to apply the desired quantity of coating smoothly to the web, the color solids are preferably adjusted so that the coating is not too viscous for easy application, nor so dilute as to be incapable of forming a tough gel. Relatively high solids content coating suspensions, e.g. of the order of 45%-65% solids or more, have been used successfully and, as a general rule, the preferred percentage of solids in the coating is governed by the type and quantity of adhesive selected for the color as set forth in the Smith application, *supra*.

The coating apparatus shown in FIGURE 1 of the drawing is a reverse roll system which has been found to be very satisfactory and effective for transferring from the trough of coating material or so-called coating color, between rolls 15 and 24, accurately controlled amounts of the coating material. With the high solids content coating colors of the order of as high as 65% solids, which in their normal condition are substantially non-flowable, this apparatus, with the rolls under considerable pressures of the order of 10 to 100 pounds per lineal inch, and with roll 24 being operated at 0.1-0.5 times the speed of application roll 15 which was turned at from 1.38-3.00 times the speed of the paper web 11, effects a large temporary

apparatus referred to, when using somewhat lower solids content colors with greatly reduced viscosity and corresponding increased flowability, has been very satisfactory in applying the desired quantity and uniform distribution of coating material to the paper web, and of leaving a surface which is sufficiently smooth so that it may be subsequently coagulated and dried on a finishing surface to give the desired high gloss coated paper. In the latter case, rolls 15, 24 are preferably operated at a low pressure of the order of 10 pounds per lineal inch, or lower and may even be operated at a gap amounting to as much as .005 inch.

Again, referring to the coating apparatus illustrated, very satisfactory results have been attained when rolls 14 and 15 were rubber covered rolls; roll 14 having a plastometer reading of about 136 P. & J. and roll 15 having a plastometer reading of about 112 P. & J. Rolls 14 and 15 may be operated with a pressure therebetween varying during operation, for example, from about 1 to 25 pounds per lineal inch, with satisfactory results having been obtained at a pressure of preferably about 10 pounds per lineal inch. Roll 24 in this connection was a hard surfaced Stonite roll. Rolls 18 and 21 had plastometer readings of 65 and 32 P. & J. respectively, while roll 20 was a metal roll, having a smoothly buffed methyl silicone casting surface, such as disclosed in co-pending application, *supra*. Roll 16 was a corrosion resistant roll such as stainless steel. More generally, however, it has been found that rolls 14, 15 and 24 may all be resilient surface type rolls, such as rubber covered rolls having a plastometer reading of the order of 80 to 140 P. & J. when measured with a  $\frac{1}{4}$  inch ball. And if one or more of these rolls is hard surfaced, i.e., of metal, Stonite, or the like, then its adjacent roll is preferably resilient surfaced. For example, the following combinations of these coating mechanism rolls have been found commercially suitable and are presented in illustration but not in limitation of the invention.

| Roll No. | Type of Roll by Combination |                  |                  |                  |             |
|----------|-----------------------------|------------------|------------------|------------------|-------------|
|          | (1)                         | (2)              | (3)              | (4)              | (5)         |
| 14-----  | Metal-----                  | 140 P. & J.----- | 136 P. & J.----- | 80 P. & J.-----  | 140 P. & J. |
| 15-----  | 112 P. & J.-----            | Metal-----       | 112 P. & J.----- | 130 P. & J.----- | Stonite.    |
| 24-----  | Metal-----                  | 112 P. & J.----- | Metal-----       | 112 P. & J.----- | 112 P. & J. |

change from its normal condition of non-flowability, causing it to become readily fluent and flowable so that it may be thus accurately controlled as to quantity and general distribution. The coating material passing in controlled amount through the nip of the rolls 15, 24 is carried on the surface of the roll 15 as it travels up toward the paper web, to transfer the desired quantity of coating material for the predetermined coat weight desired, and in such condition of flowability that the color will be generally distributed across the surface of the roll 15 as it moves toward the paper and application nip of rolls 15, 14. In such condition of flowability and such distribution that when brought in contact with the paper web by roll 15 turning in a direction opposite to the direction of travel of the paper web, there will be transferred to the web a substantially uniformly distributed layer or film of coating material which is of considerable and unexpected smoothness. The coating materials commonly used, contain a substantial amount of adhesive material such as casein. However, by the disclosed reverse roll system, there is sufficient working of the coating color both before it passes into the application nip of the rolls 14, 15, and also within the nip by reason of the reverse turning of roll 15, so that even high solids content coating colors will be made sufficiently fluid, for securing the desired accurate coat weight and the uniform distribution of the film upon the surface of the paper web. Moreover, the

50 All plastometer values were measured with a  $\frac{1}{4}$  inch P. & J. ball. Whenever the surface of the application roll 15 is provided with a resilient cover, as in Examples 1, 3, and 4 above, it is desirable to operate the coater in a manner such that the film of coating on roll 15 is only partially transferred to the web of paper, and the 55 excess serves as a lubricating layer to prevent excessive drag between the paper web and the surface of roll 15. The presence of this lubricating layer is a normal occurrence under the operating conditions previously specified.

60 The pressure in operation between rolls 18 and 20 may be varied over a substantial range; for example, from about 200 to 600 pounds per lineal inch, with satisfactory results having been obtained at a pressure of about 400 pounds per lineal inch. In this connection, it has been found that the upper pressure limit is determined by the strength or toughness of the gelled coating. And the pressure between rolls 18 and 20 may be varied over wide limits so long as sufficient pressure is used to insure intimate contact between the coating surface and the casting surface.

65 Various coating materials may be employed in practicing the present invention and as indicated by the formulations hereinafter set forth, the coating material generally comprises a mineral and an adhesive in aqueous medium. Both the adhesive content and the total solids content of the coating materials to be used are predicated on the

ultimate high gloss coated paper desired and for highly satisfactory operations, such adhesive and total solids content may be somewhat critical. For example, it has been found that the preferred range of adhesive contents is of the order of 12%-20%, although more or less adhesive can be used if special end-use requirements of the ultimate high gloss paper product so dictate. Moreover, if starch is used in admixture in the adhesive, more total adhesive is required than if it is not so used. Generally, the higher region of the adhesive content range is useful in preparing papers for offset printing, while the lower range has been found useful for letterpress printing.

A color formula which has been found to function satisfactorily in the practicing of the invention is of the following composition, wherein the parts by weight are taken on a dry basis:

*Example I*

|                                                                                                            | Parts by weight |
|------------------------------------------------------------------------------------------------------------|-----------------|
| Clay (English coating clay)                                                                                | 42.0            |
| Calcium carbonate                                                                                          | 42.0            |
| Casein (Argentina)                                                                                         | 12.0            |
| Caustic soda (parts per 100 parts of casein)                                                               | 6.0             |
| Sodium pyrophosphate                                                                                       | 0.75            |
| Calcium stearate                                                                                           | 0.5             |
| Dow 512-R latex (butadiene-styrene copolymer 30:70)                                                        | 6.0             |
| Di-isobutylphenoxyethoxyethylidemethylbenzyl ammoniumchloride, monohydrate (Hyamine 1622, Rohm & Haas Co.) | 0.05            |

Such color gives satisfactory results in the practicing of this invention when admixed with water to have a solids content of approximately 50.5%.

The following examples of color formulations which have likewise been used satisfactorily are set for purposes of illustration, but not of limitation. The parts by weight of these compositions are taken on a dry basis:

*Example II*

|                                                 | Parts by weight |
|-------------------------------------------------|-----------------|
| Clay (English coating clay)                     | 42.0            |
| Calcium carbonate                               | 42.0            |
| Soya protein (refined)                          | 12.0            |
| Ammonia-26° Bé (parts per 100 parts of protein) | 12.0            |
| Dow 512-R latex                                 | 4.0             |
| Sodium pyrophosphate                            | 0.75            |
| Calcium stearate                                | 0.5             |
| Hyamine 1622                                    | 0.05            |

*Example III*

|                                                 | Parts by weight |
|-------------------------------------------------|-----------------|
| Clay (English coating clay)                     | 38.0            |
| Calcium carbonate                               | 41.0            |
| Satin white                                     | 5.0             |
| Alpha protein                                   | 12.0            |
| Ammonia-26° Bé (parts per 100 parts of protein) | 12.0            |
| Dow 512-R latex                                 | 4.0             |
| Sodium pyrophosphate                            | 0.75            |
| Calcium stearate                                | 0.5             |
| Lignasan                                        | 0.05            |

*Example IV*

|                                                        | Parts by weight |
|--------------------------------------------------------|-----------------|
| Clay (English coating clay)                            | 51.0            |
| Calcium carbonate                                      | 30.0            |
| Alpha protein                                          | 18.0            |
| Azite (dicyandiamide) (parts per 100 parts of protein) | 25.0            |
| Ammonia-26° Bé (parts per 100 parts of protein)        | 12.0            |
| Sodium pyrophosphate                                   | 0.75            |
| Calcium stearate                                       | 0.5             |
| Lignasan                                               | 0.05            |

*Example V*

|                                                 | Parts by weight |
|-------------------------------------------------|-----------------|
| Calcium carbonate                               | 84.0            |
| Alpha protein                                   | 12.0            |
| Ammonia-26° Bé (parts per 100 parts of protein) | 18.0            |
| Dow 512-R latex                                 | 4.0             |
| Sodium pyrophosphate                            | 0.75            |
| Calcium stearate                                | 0.5             |
| Hyamine 1622                                    | 0.05            |

*Example VI*

|                                                        | Parts by weight |
|--------------------------------------------------------|-----------------|
| Clay (domestic coating clay)                           | 81.0            |
| Soya protein (refined)                                 | 12.0            |
| Azite (dicyandiamide) (parts per 100 parts of protein) | 25.0            |
| Ammonia-26° Bé (parts per 100 parts of protein)        | 15.0            |
| Sodium pyrophosphate                                   | 0.75            |
| Sulphonated tallow (vegtol)                            | 1.0             |
| Calcium stearate                                       | 0.5             |
| Dow 512-R latex                                        | 7.0             |
| Hyamine 1622                                           | 0.1             |

The surface temperature of the casting drum 20 which preferably is a chromium surfaced roll and is preferably from 80° C. to 101° C. during the drying cycle for producing the cast-surfaced coated paper having unusually high brightness and opacity and high gloss of this invention, although temperatures ranging from 65° C. to as high as 105° C. have been used without harmful results. It has been found that temperatures approaching 90-101° C. are advantageous when the more active coagulants are employed.

In the coater modification shown in FIGURE 2, rolls 32 and 33 form the metering pair of the coater. One or both of these rolls are provided with a resilient surface, such as a rubber cover. They may be operated at equal speeds, or roll 33 may be rotated more slowly than roll 32. They rotate in opposite angular directions, as indicated by arrows and the pressure between these rolls is controllable. When a film of coating from pool 34 is metered between rolls 32 and 33, a portion of this film follows the face of roll 32 into contact with roll 31 where it is blended in the nip formed by rolls 31 and 32. Roll 31 may be operated more slowly, equal to or faster than roll 32, and is preferably operated with a surface speed greater than that of roll 30.

Roll 31 can be made of rubber or some other resilient material, but preferably, it has a hard, abrasive-resistant surface, such as brass, chromium or Stonite. Roll 31 transfers a part of the coating from the face of roll 32 and applies it to the paper wrapping roll 30, with a wiping action. The surface of roll 31 must be relatively smooth in comparison to the thickness of the film it carries. And, if desired, a smoothing device 35 such as a flexible distributor or a spread shaft may be installed in the position shown in FIGURE 2, so that it lightly contacts the surface of roll 31 and smoothes the coating on this surface. If a shaft is used instead of a spring steel type distributor, it should be made of a material permitting satisfactory contact with the surface of roll 31. For example, if roll 31 has a hard surface, the spread shaft should be rubber covered. Such a smoothing device, while not always necessary, may be desirable in cases where the film pattern produced by the splitting of the wet film in the nips between rolls 32 and 33 or between rolls 31 and 32 is being transferred without adequate blending to the paper in the nip between rolls 30 and 31.

It has been found that the coater described and shown in FIGURE 2 of the drawing, provides a unique combination or precise coat weight control, unrestricted coat weight level and excellent smoothness of the coated surface and coverage of the rawstock in the production of high gloss cast-surfaced mineral coated papers.

While the methods, apparatus and products herein described are for the purpose of illustration only, it is to be understood that the present invention includes all modifications and equivalents which fall within the scope of the invention which is defined by the appended claims.

What is claimed is:

1. Web coating apparatus comprising a coating roll, means for conveying a web to be coated to and from said coating roll, a metering roll mounted with the axis thereof in substantially the same horizontal plane as the axis of said coating roll to form with said coating roll a metering nip, means for maintaining a pool of coating material adjacent an upper nip formed by the contact relationship of the metering and coating rolls, at least one of said rolls forming said metering nip being resiliently surfaced, said rolls being in abutting relation under a pressure of the order of 0 to 100 pounds per lineal inch, means for rotating said rolls in the same predetermined angular direction to cause relative reverse rotation of said rolls and also to cause the surface of said coating roll to move upwardly in a direction opposite to the direction of the web.

2. Web coating apparatus comprising a coating roll, means for conveying a web to be coated to and from said coating roll, a metering roll mounted with the axis thereof in substantially the same horizontal plane as the axis of said coating roll to form with said coating roll a metering nip, means for maintaining a pool of coating material adjacent an upper nip formed by the contact relationship of the metering and coating rolls, at least one of said rolls forming said metering nip being resiliently surfaced, said rolls being in abutting relation under a pressure of the order of 0 to 100 pounds per lineal inch, means for rotating said rolls in the same predetermined angular direction to cause relative reverse rotation of said rolls and also to cause the surface of said coating roll to move upwardly in a direction opposite to the direction of the web and in wiping contact therewith.

3. Web coating apparatus comprising an applicator roll, a backing roll forming an application nip with said applicator roll, and said application nip adapted to pass therethrough a web to be coated, a metering roll mounted with the axis thereof in substantially the same horizontal plane as the axis of said applicator roll to form with said applicator roll a metering nip, means for maintaining a pool of coating material above said metering nip, said rolls being in an abutting relationship under a pressure of the order of 0 to 100 pounds per lineal inch, one of said rolls forming said metering nip having a resilient surface, one of said rolls forming said application nip having a resilient surface, means for rotating said rolls in the same predetermined angular direction to cause relative reverse travel of the surfaces thereof and to cause said surface of said applicator roll to move in the direction opposite the direction of the web.

4. Web coating apparatus comprising a plurality of rolls, said rolls forming a metering nip, a blending nip and an application nip, said application nip adapted to pass therethrough a web to be coated, said rolls forming said metering nip being in abutting relationship and under a pressure of the order of 0 to 100 pounds per lineal inch, at least one of said rolls forming said metering nip having a resilient surface, means for maintaining a pool of coating material above said metering nip, means for rotating said rolls forming said blending nip in the same predetermined angular direction, means for rotating said rolls forming said application nip in the same predetermined angular direction to cause relative reverse travel of the surfaces thereof.

5. A process for producing cast-surfaced mineral coated paper wherein a continuously moving web of paper is smoothly and evenly coated with a coating suspension which is later brought to a high gloss by passing the

coated web over and in intimate contact with the surface of a finishing roll, which comprises, prior to casting: applying a mineral-adhesive coating suspension having from about 45% to about 65% total solids to a pressure nip formed between the surface of a metering roll and the surface of an applicator roll, the pressure between said rolls being of the order of 0 to 100 pounds per lineal inch, and at least one of said rolls having a resilient surface, said metering roll and said applicator roll moving in the same angular direction, said applicator roll surface engaging said web and moving in the opposite direction thereto, transferring a portion of said coating suspension from said applicator roll to said web while retaining a portion thereof on said moving applicator roll surface whereby a lubricating film of said coating is maintained on said applicator roll surface.

6. A process for producing cast-surfaced mineral coated paper wherein a continuously moving web of paper is smoothly and evenly coated with a coating suspension which is later brought to a high gloss by passing the coated web over and in intimate contact with the surface of a finishing roll, which comprises, prior to casting: applying a mineral-adhesive coating suspension having from about 45% to about 65% total solids to a pressure nip formed between the surface of a metering roll and the surface of an applicator roll, one of said rolls having a hard surface and the other of said rolls having a resilient surface, said metering roll and said applicator roll moving in the same angular direction, said applicator roll surface engaging said web and moving in the opposite direction thereto, transferring a portion of said coating suspension from said applicator roll to said web while retaining a portion thereof on said moving applicator roll surface whereby a lubricating film of said coating is maintained on said applicator roll surface.

7. A process for producing cast-surfaced mineral coated paper wherein a continuously moving web of paper is smoothly and evenly coated with a coating suspension which is later brought to a high gloss by passing the coated web over and in intimate contact with the surface of a finishing roll, which comprises, prior to casting: applying a mineral-adhesive coating suspension having from about 45% to about 65% total solids to a pressure nip formed between the surface of a metering roll and the surface of an applicator roll, one of said rolls having a hard surface and the other of said rolls having a resilient surface, the pressure between said rolls being of the order of 0 to 100 pounds per lineal inch, said metering roll and said applicator roll moving in the same angular direction, said applicator roll surface engaging said web and moving in the opposite direction thereto, transferring a portion of said coating suspension from said applicator roll to said web while retaining a portion thereof on said moving applicator roll surface whereby a lubricating film of said coating is maintained on said applicator roll surface.

#### References Cited by the Examiner

#### UNITED STATES PATENTS

|    |           |         |                  |       |           |
|----|-----------|---------|------------------|-------|-----------|
| 60 | 1,508,720 | 9/1924  | Perry            | ----- | 117—64    |
|    | 2,157,212 | 5/1939  | Moore            | ----- | 117—111   |
|    | 2,185,859 | 1/1940  | Massey           | ----- | 117—111   |
|    | 2,199,228 | 4/1940  | Obenshain et al. | ----- | 117—64    |
|    | 2,252,345 | 8/1941  | Johnson          | ----- | 117—64    |
| 65 | 2,678,890 | 5/1954  | Leighton         | ----- | 117—64    |
|    | 2,829,980 | 4/1958  | Redd             | ----- | 117—64    |
|    | 2,842,092 | 7/1958  | Pomper           | ----- | 117—111 X |
|    | 2,870,738 | 1/1959  | Jacobs et al.    | ----- | 118—249   |
|    | 2,919,205 | 12/1959 | Hart             | ----- | 117—64    |

WILLIAM D. MARTIN, Primary Examiner.

MURRAY KATZ, RICHARD D. NEVIUS, Examiners,